

## UNITED STATES PATENT OFFICE

2,373,278

COATED ARTICLE AND METHOD OF  
PRODUCTION THEREOFWaldorf S. Traylor, Newport, Del., assignor to  
Hercules Powder Company, Wilmington, Del., a  
corporation of DelawareNo Drawing. Application June 27, 1941,  
Serial No. 400,120

7 Claims. (Cl. 117—65)

This invention relates to an improved coated textile material and to a method of production thereof.

The coating of textile fabrics to provide such products as artificial leather and similar coated fabrics has been practiced for many years utilizing lacquers and heavy nitrocellulose dope solutions as the coating agents. Repeated coatings have been required to build up the desired thickness of coating since there is a definite limit to the thickness of coating which can be applied at one time. The operation is usually carried out by applying a first coating to the fabric and then drying the coating to remove the solvents and then repeating the operation successively until the proper thickness of coating is obtained. In the production of artificial leather it is usually necessary to apply at least about seven separate coats to the fabric. It is apparent that considerable handling of the fabric is therefore necessary and the operation is consequently quite costly. The volatile solvents which are used introduce serious fire hazards and also require use of solvent recovery systems to make the operation economically feasible. A high proportion of plasticizer has always been necessary with the nitrocellulose to provide sufficient flexibility of the coating. In fact, as much plasticizer as the coating will tolerate without spewing at slightly elevated temperatures is usually included in the formula. Such large amounts of plasticizer are necessary in the lacquer dopes since the dopes penetrate the material being coated and tend to stiffen it more than desired. To avoid such stiffening the first coats are generally plasticized more heavily than the subsequent coats, and such coats are quite tacky.

It is an object of this invention to provide an improved method of coating textile fabrics.

It is another object to provide an improved method of coating textile fabrics which requires only one coating operation.

It is a further object to provide an improved method of coating textile fabrics which eliminates the use of volatile organic solvents.

Another object of the invention is to provide an improved coated textile fabric.

The above objects may be accomplished in accordance with this invention by applying a plastic composition free of organic solvents and comprising ethyl cellulose and a plasticizer therefor to a textile fabric by means of heat and pressure. Application of the plastic to the fabric may be carried out by means of heated power rolls, such 55

as for example a two roll plastic mill or a calender stack composed of three or more rolls. Since no solvents are present, the plastic composition does not impregnate the fabric to any observable extent. However, the heat and pressure which are applied to the plastic to make it flow cause it to penetrate the fabric only sufficiently to anchor the coating and insufficient to cause immobilization of the individual threads or fibers. Consequently no stiffening of the fabric occurs.

With use of other film formers heretofore used for coating cloth, such as for example nitrocellulose, solvents have been necessary due to the non-thermoplastic nature of the nitrocellulose. Use of a small enough amount of solvent to prevent impregnation has not been possible and still insure flowability. Ethyl cellulose, being truly thermoplastic in character, is ideally adapted to application without use of solvents and thus makes possible the improvements in textile fabric coating described in accordance with this invention.

While ethyl cellulose may be used alone in the process of the invention, it will usually be desirable to include a plasticizer for the ethyl cellulose to provide coated fabrics having the most satisfactory characteristics.

The ethyl cellulose which is utilized in the compositions of this invention is the type which has an ethoxyl content in the range from about 41% to about 51%, and preferably from about 44% to about 49%. The viscosity characteristic may vary widely and will usually be above about 7 centipoises and preferably between about 70 and 300 centipoises, as measured on a 5% solution in a solvent consisting of 70% toluene and 30% denatured ethyl alcohol.

As plasticizers the compositions utilized may include dibutyl phthalate, tricresyl phosphate, methyl phthalyl ethyl glycolate, chlorinated diphenyls, refined mineral oil, raw or air blown castor oil, soya bean oil, acetyl triethyl citrate, long oil-modified alkyd resins containing over 60% of combined oil or fatty acid, etc. The amount of plasticizer will vary with the particular plasticizer, with the properties desired in the final coating and with the viscosity of the ethyl cellulose employed. The amount of plasticizer will generally not exceed about 60% by weight of the composition.

Small amounts of modifying agents may be included in the compositions if desired. A small amount of a wax, not to exceed about 3.5 per cent may be included to improve water-resisting prop-

erties. The amount of wax included will in no case be sufficient to interfere with adhesion of the coating. With Japan wax, for example, 3.5% is the maximum amount utilizable, while no more than 1 per cent of paraffin wax or 0.5 per cent of carnauba wax can be included without being seriously detrimental to adhesion. Fillers, pigments, or dyestuffs may be included if desired.

The plastic compositions utilized in the invention may be prepared by mixing the ingredients in lump or powder form and colloidizing on heated rolls, heated Banbury mill or other suitable device for compounding plastic substances without use of solvents. The temperature employed in compounding the plastic will be sufficient to render the composition flowable and will usually be from about 90° C. to about 150° C.

In applying the plastic composition to a textile fabric in accordance with the method of the invention the details of the operation will vary with the particular coating device employed. In general, however, the molten plastic composition in homogeneous condition will be applied by means of rolls to the textile fabric using heat and pressure sufficient to flow the composition onto the fabric. The adjustment of the opening between the rolls will control the thickness of coating applied to the fabric. The fabric emerges from the nip of the coating roll uniformly coated with an adherent and flexible coating of any desired thickness. For example, in a heated two roll mill the plastic composition is worked on the rolls until thoroughly softened and distributed on one roll and in amount sufficient to form a uniform bead in the nip. With proper adjustment of the rolls to provide the desired thickness of the plastic on the roll and with the temperature sufficiently high to render the bead fluid and shiny, the textile fabric is threaded through the nip. Emerging from the nip it will be coated uniformly with the plastic and may be cooled to set the coating.

With use of a calender stack in place of the two roll mill the coating principle will be the same. It will be desirable to preheat the fabric to the coating temperature prior to coating with the plastic composition and this can be done readily in the multiple roll calender stacks. The temperature of application of the plastic will generally fall within the range of about 90° C. to about 150° C. The specific temperature employed with any specific composition will be determined by the nature of the composition in question.

The coated textile fabric obtained as a result of the coating operation of the invention will be characterized as having a flexible coating tightly adhering to the surface of the fabric with substantially no impregnation thereof and will have a coating thickness varying from a minimum of about one mil to a maximum of about 100 mils. It will be suitable for such purposes as artificial leather, window shade cloth, waterproof wrappings, substitute for oil cloth, etc.

The various embodiments of the invention are illustrated by the following specific examples:

#### Example I

A mixture of 75 parts by weight of ethyl cellulose having an ethoxyl content of about 48 per cent and a viscosity of about 100 centipoises, 75 parts of pale blown castor oil and 19 parts of chlorinated diphenyl was compounded on a heated two roll mill until uniformly heated and distributed on one roll and a cloth then fed through the nip. A coated cloth having a uni-

form and smooth flexible coating of about 15 mils thickness resulted.

#### Example II

5 The procedure of Example I was repeated with use of a composition consisting of 180 parts by weight of ethyl cellulose of about 48 per cent ethoxyl and about 100 centipoises viscosity and 10 120 parts by weight of chlorinated diphenyl. A similarly coated fabric resulted.

#### Example III

A mixture composed of 77 parts by weight of 15 ethyl cellulose having an ethoxyl content of about 48 per cent and a viscosity of about 300 centipoises, 23 parts by weight of refined mineral oil, 0.06 part by weight of Sudan Yellow dye, and 0.25 part by weight of titanium dioxide was milled on a heated two-roll mill at a temperature of about 300° F. until the composition was uniformly heated and distributed on one roll. A cotton duck fabric preheated to 300° F. was then fed through the nip and was coated uniformly with a flexible and adherent coating of the composition of about 10 mils thickness.

25 It will be understood that the details and examples hereinbefore set forth are illustrative only, and that the invention as broadly described and claimed is in no way limited thereby.

30 What I claim and desire to protect by Letters Patent is:

1. The method of coating a textile fabric to provide a tightly adherent, flexible coating on the surface with substantially no impregnation thereof, which comprises applying to a textile fabric 35 a molten plastic composition consisting of ethyl cellulose, a plasticizer therefor and from 0 to about 3.5% by weight of a wax as the film-forming components under heat and pressure sufficient to cause it to flow, then allowing the fabric to cool.

2. The method of coating a textile fabric to provide a tightly adherent, flexible coating on the surface with substantially no impregnation thereof, 45 which comprises applying to a textile fabric a molten plastic composition consisting of ethyl cellulose, a plasticizer therefor and from 0 to about 3.5% by weight of a wax as the film-forming components at a temperature of about 50 90° to about 150° C. under pressure, then allowing the fabric to cool.

3. The method of coating a textile fabric to provide a tightly adherent, flexible coating on the surface with substantially no impregnation thereof, 55 which comprises applying to a textile fabric a molten plastic composition consisting of ethyl cellulose, a plasticizer therefor in an amount not in excess of about 60% by weight, and from 0 to about 3.5% by weight of a wax as the film-forming components at a temperature of about 90° to 60 about 150° C. under pressure, then allowing the fabric to cool.

4. A textile fabric carrying a tightly adherent, 65 flexible surface coating applied thereto without substantial impregnation thereof, of a plastic composition consisting of ethyl cellulose, a plasticizer therefor and from 0 to about 3.5% by weight of a wax as the film-forming components, said coating having a thickness from about one mil to about 100 mils.

5. A textile fabric carrying a tightly adherent, 70 flexible surface coating applied thereto without substantial impregnation thereof, of a plastic composition consisting of ethyl cellulose, a plasticizer therefor in an amount not in excess of

about 60% by weight, and from 0 to about 3.5% by weight of a wax as the film-forming components, said coating having a thickness from about one mil to about 100 mils.

6. A textile fabric carrying a tightly adherent, flexible surface coating applied thereto without substantial impregnation thereof, of a plastic composition consisting of ethyl cellulose and chlorinated diphenyl, said coating having a thickness from about one mil to about 100 mils. 10

7. A textile fabric carrying a tightly adherent, flexible surface coating applied thereto without substantial impregnation thereof, of a plastic composition consisting of ethyl cellulose and blown castor oil, said coating having a thickness from about one mil to about 100 mils.

WALDORF S. TRAYLOR.